

## UNITED STATES PATENT OFFICE

HAROLD R. RAFTON, OF LAWRENCE, MASSACHUSETTS, ASSIGNOR TO RAFFOLD PROCESS CORPORATION, A CORPORATION OF MASSACHUSETTS

## MANUFACTURE OF PAPER

No Drawing.

Application filed November 27, 1928. Serial No. 322,291.

This invention relates to the manufacture of paper.

The principal object of my invention is to provide a method whereby paper may be manufactured to contain an amount of filler greater than is feasible by the usual procedure.

An important object is to provide a method whereby in the papermaking operation a smaller proportion of the filler than is normal passes through the web-forming device into the white water.

A further object is to provide a method whereby paper of very high filler content may be manufactured.

Other objects and advantages of my invention will become apparent in the course of the following description.

The ordinary method of manufacturing paper is to mix the fibre and filler in the beater or like machine, together with alum, or alum and size, and then after suitable treatment in the beater, to pass the mix through the subsequent apparatus and mechanical 25 treating equipment such as the chests and the jordan, and then to dilute the mix at the mixing box with white water, e. g. tray water from the machine, and with other water if desired, and finally to conduct the diluted 30 mix to the web-forming device of the paper machine. Here the web is formed with simultaneous removal of the white water, which normally contains a relatively larger proportion of filler to fibre than does the 35 stock fed to the web-forming device.

The retention of filler in paper has always been a matter for serious consideration in papermaking. In the former prevailing practice, which has now been superseded to 40 a considerable extent, practically all of the white water (excepting part of the tray water) flowed to waste and hence a considerable proportion of the filler employed in the beater escaped in the white water and was lost. 45 This condition was greatly improved by the introduction of save-all systems, such as by sedimentation, filtration, deckering, or the like which usually recover a large proportion, and in some cases practically all, of 50 the solids suspended in the white water.

Such save-all systems usually return the recovered stock to the beater or to one of the chests for re-use in the cycle. This practice has thus eliminated to a considerable extent the wastage of filler. It has consequently reduced the amount of filler required to be used in the beater for a given filler content in the paper. Moreover it has provided a means by which a relatively higher percentage of filler in the finished paper may be obtained in regular commercial production than was formerly feasible, as it is now possible to carry a higher percentage of filler to fibre circulating in the machine waters without excessive losses.

However even with the present save-all systems there is a practical limit to which the filler content of paper may be raised for any given set of conditions. This results from the fact that when the filler content of 70 the stock is pushed beyond a certain point the paper web will not hold appreciably more filler, and moreover under these conditions the save-all systems rapidly become inefficient and fail to recover the greatly increased 75 filler content of the white water.

For instance in magazine paper, with a sulphite-soda furnish, with several hours beating, and machine speed between 350 and 400 feet per minute, using a sedimentation 80 save-all system, the filler content runs about 22% as a maximum. With a furnish consisting of approximately equal parts of sulphite pulp, soda pulp and old paper stock with from 1 to 2 hours beating, with a machine 85 speed of approximately 400 feet per minute, using a filtration save-all system, the filler content runs about 24% as a maximum.

It will be understood, of course, that with varying conditions of hydration of the stock, and varying kinds of fibre and grades of paper to be made as well as varying machine speeds, amounts of sizing, alum, and the variation of the numerous other factors in 95 papermaking, that the filler content in any given case may vary somewhat one way or the other, but in making, for instance, a magazine grade of paper the above represent approximately the maximum filler contents 100

which can be obtained in regular machine operation.

I have discovered that it is possible to increase the filler content of paper, above that percentage normally obtainable when the usual method is employed, by the expedient of adding alum to the paper mix at or subsequent to the point at which the mix is diluted prior to delivery to the web-forming device, 10 that is, in other words, at the wet end of the paper machine.

I have found for instance that a given amount of alum added in the beater to a fibrous mix containing filler will not produce 15 a paper having as high a filler content as will an equal amount of alum added at the wet end of the paper machine to a similar fibrous-filler mix. The difference may range from 20 as low as 1% in some cases up to 3 or 4% in other cases, and in still other cases the difference in percentage may be much higher. Even the lower mentioned difference of 1% 25 is of great economic importance, amounting to a saving of \$30 to \$50 per day in a 100 ton mill (assuming no change in fibre furnish), and of course the saving mounts proportionately with the increase of the difference in 30 filler content that it is possible to obtain.

Of course part of the alum may be added 35 in the beater and part at the wet end of the paper machine, but I have found that the maximum results are obtained by the use of all the alum at the wet end of the paper machine.

In the practice of my invention my preferred method is to add the fibrous materials and filler, together with size if any is to be employed, in the beater, subject the mix to the usual mechanical treatment, then pass it 40 through the usual steps and mechanical treating machinery up to the point at which it is to be diluted prior to the delivery to the web-forming device. At or subsequent to 45 this point I add the requisite amount of alum, preferably continuously, preferably in dilute aqueous solution, either in fresh water, or admixed with a diluting liquid.

I have found that if the alum be added 50 when the fibrous mix containing the filler is in relatively concentrated condition, even after it has left the beater, and particularly in places where the mix would be subjected to agitation such as is normal in the stuff chests, 55 this effect of increased filler retention is deteriorated, and thus to procure the effect it is necessary to add the alum under such conditions that there is a minimum of intimacy as well as time of contact of the constituents of 60 the mix, namely, at the wet end of the paper machine. I have also found that prolonged agitation even in the dilute state injures the effect, but from a practical standpoint the time that the mix remains in the dilute condition in the ordinary papermaking procedure 65

is not sufficient to deteriorate substantially the effect I obtain.

Of course if desired the filler as well as the size may also be added at the wet end of the paper machine, but the important point is that the alum must be added at this point, and I therefore consider the addition of the filler and size together with the alum at this point the equivalent of adding the 70 filler and size to the fibre in the beater. I have not found that the presence of sizing 75 has any marked effect on the filler retention when my process is employed. The alum seems to be the controlling factor.

My process results in a greater retention of 80 filler in the paper and hence, under any given set of circumstances, in a smaller amount of filler passing through into the white water, with a corresponding lessened 85 difficulty in operating save-all systems. Of course, to obtain a higher filler content in the paper than formerly, where a substantially closed white water cycle is employed, more 90 filler in proportion to fibre than formerly should be used in the furnish.

In the above description of my preferred 95 practice I have assumed a use of alum no greater than that regularly employed under any given set of conditions. However, I have found that it is sometimes very desirable 100 to increase this amount of alum, and thereby still further increase the percentage of filler retained in the paper. The saving obtained by increased filler content normally more than offsets the increased alum cost. This increased use of alum is indicated up to 105 the point where other factors negative the desirability of further increased filler content, such as strength, two-sidedness, or the like. The amount of extra alum which is desirable to be added may also be limited to some extent by the desire not to get the stock too acid.

Instead of alum, I may use other salts of 110 aluminum such as the chloride, or with a certain measure of success, other metallic salts such as zinc salts, for example zinc sulphate.

By the word "filler" I mean such inorganic 115 loading as clay, talc, or the like, which is insoluble in water and substantially chemically inert to the materials ordinarily employed in papermaking, such for example as alum.

By the words "filled paper" I mean paper filled with material coming under the definition of the word "filler" given above.

When I use the word "paper" herein, I 120 use it in the broad sense to include products of manufacture of all types and of all weights and thicknesses, which contain as an essential constituent a considerable amount of prepared fibre and which are capable of 125 being produced on a Fourdrinier, cylinder, 130

or other forming, felting, shaping or molding machine.

By the term "wet end of the paper machine" I intend to include those instrumentalities employed in paper manufacture by which and/or in which a relatively concentrated paper mix is diluted, and treated, conveyed or fed up to the point of web-formation, such as the mixing box, regulating and proportioning devices, rifiers, troughs, screens, head boxes, inlets, and the like.

While I have described in detail the preferred embodiment of my invention, it is of course to be taken as illustrative only and not limiting, as it is to be understood that details of procedure, kinds of material used in furnishes, proportions of ingredients, and arrangement of steps may be widely varied without departing from the spirit of my invention or the scope of the subjoined claims.

I claim:

1. The method of producing filled paper, comprising adding a metallic salt to a mix comprising fibrous material and filler under conditions favoring the minimizing of time of contact, and thereafter making paper therefrom.

2. The method of producing filled paper, comprising adding a metallic salt to a mix comprising fibrous material and filler under conditions favoring the minimizing of intimacy and time of contact, and thereafter making paper therefrom.

3. The method of producing filled paper, comprising adding a metallic salt at the wet end of the paper machine to a mix comprising fibrous material and filler, and thereafter making paper therefrom.

4. The method of producing filled paper, comprising adding a salt of aluminum at the wet end of the paper machine to a mix comprising fibrous material and filler, and thereafter making paper therefrom.

5. The method of producing filled paper, comprising adding alum at the wet end of the paper machine to a mix comprising fibrous material and filler, and thereafter making paper therefrom.

6. The method of producing filled paper, comprising adding a metallic salt at the wet end of the paper machine to a mix comprising fibrous material consisting of sulphite pulp and soda pulp and filler, and thereafter making paper therefrom.

7. The method of producing filled paper, comprising adding a metallic salt at the wet end of the paper machine to a mix comprising fibrous material consisting of sulphite pulp, soda pulp, and old paper stock and filler, and thereafter making paper therefrom.

8. The method of producing filled paper comprising mixing fibrous material and filler in a beater, adding a metallic salt at the wet end of the paper machine, and thereafter making paper therefrom.

9. The method of producing filled paper comprising mixing fibrous material and filler in a beater, adding a salt of aluminum at the wet end of the paper machine, and thereafter making paper therefrom.

10. The method of producing filled paper comprising mixing fibrous material and filler in a beater, adding alum at the wet end of the paper machine, and thereafter making paper therefrom.

In testimony whereof I affix my signature.

HAROLD ROBERT RAFTON.

70

75

80

85

90

95

100

105

110

115

120

125